

# UNITED STATES PATENT OFFICE.

JOHN COUP, OF MARION, OHIO.

## NON-CORROSIVE METALLIC ALLOY.

1,069,113.

Specification of Letters Patent.

Patented Aug. 5, 1913.

No Drawing.

Application filed April 1, 1913. Serial No. 758,232.

*To all whom it may concern:*

Be it known that I, JOHN COUP, a citizen of the United States, residing at Marion, in the county of Marion and State of Ohio, have invented certain new and useful Improvements in Non-Corrosive Metallic Alloys, of which the following is a specification.

This invention relates to an improved metal alloy and has for its primary object to provide a composition consisting of a number of mineral constituents homogeneously commingled or mixed with a suitable deoxidizing agent whereby a metal alloy is produced which may be utilized as a substitute for nickel-plating and may be commercially used in the manufacture of various articles.

Another object of the invention is to produce a metal alloy which has great strength and durability, may be inexpensively compounded and is particularly desirable and serviceable in the manufacture of piano strings, bells and similar articles wherein it is essential that the metal be noncorrosive in order to preserve the tone qualities thereof.

With the above and other objects in view as will become apparent as the description proceeds, the invention consists in the combination of the several mineral ingredients hereinabove specified, mixed and treated in the manner set forth.

The constituents of my improved alloy are as follows:

|    |              |              |
|----|--------------|--------------|
| 35 | Copper       | 69.13 parts, |
|    | Nickel       | 14.81 parts, |
|    | Zinc         | 8.64 parts,  |
|    | Aluminum     | 3.70 parts,  |
|    | Phosphor-tin | 3.08 parts,  |
| 40 | Lead         | .58 parts,   |
|    | Iron         | .06 parts.   |

In the preparation of the alloy, the copper iron and nickel are first placed in a pot and inserted in a crucible. These two ingredients are heated to about 3080 degrees Fahrenheit, at which point they are liquefied or melted. The heat is then reduced to about 700 degrees Fahrenheit and the zinc is now added in small quantities. After these ingredients have become thoroughly commingled, the lead is added. The heat is reduced to about 400 degrees Fahrenheit

just prior to removing the pot, and the phosphor tin is then added to the mixture. The addition of this last ingredient destroys all the corrosive acids in the copper, zinc and nickel. During the preparation of the alloy, the compound is kept well covered with charcoal. After removing the pot from the crucible, the dross is skimmed from the surface of the mixture and the aluminum is added. The aluminum acts as a deoxidizing agent for the other ingredients.

The metal alloy produced in the manner above described is adapted for general commercial use. In using the same in the manufacture of cast articles, dry sand is used in the mold and while the metal is being poured, all windows, doors and other openings are closed to prevent drafts and thereby obviate oxidizing of the metal which should be poured quickly while at a white heat. Phosphor-tin constitutes the base of my new metal, but when the compound is used for the manufacture of knives or other articles which are stamped or cut out, the quantity of tin is increased and the quantity of phosphorus is decreased. Conversely, in the use of the compound for the manufacture of articles which require rolling, the tin is greatly reduced and in some instances altogether omitted. The use of the phosphor-tin results in the production of a metal alloy which is malleable while at the same time being extremely strong and durable. The product which is procured by combining the several mineral ingredients in the manner above described is absolutely non-corrosive and may be rolled into sheets and drawn. The metal may be used in the manufacture of various articles of cutlery, harness trimming, automobile trimmings, soda fountains, as a metal packing, and for many other uses.

In subjecting this improved metal to a test, it has been found that the same has a tensile strength of from seventy to ninety thousand pounds to the square inch and a torsional strength of about forty-five thousand pounds.

Owing to the fact that the metal alloy is non-corrosive the same is especially desirable for the manufacture of bells, and strings for pianos and other musical instruments where it is essential that the tone

qualities be preserved. The alloy also provides a very satisfactory substitute for nickel-plating and may be produced at about the cost of a good quality of brass.

From the foregoing it is thought that the manner of compounding my improved metal alloy and the several advantages thereof will be clearly understood. As the same consists of but few ingredients, it will be seen that any desirable quantity of the alloy may be quickly produced. The proportions of the several ingredients hereinbefore stated should be faithfully adhered to as the same has been found to produce the best results in

the use of the metal for commercial purposes. 15

What I claim is:

A metal alloy consisting of copper, 69.13 per cent., nickel, 14.81 per cent., zinc, 8.64 per cent., lead, .58 per cent., iron, .06 per cent., phosphor-tin, 3.08 per cent. and aluminum, 3.70 per cent. 20

In testimony whereof I hereunto affix my signature in the presence of two witnesses.

JOHN COUP.

Witnesses:

CHARLES MILLER BENDER,  
LIDA MAY BENDER.